

## UNITED STATES PATENT OFFICE

2,581,076

DECORATED WALLBOARD AND METHOD OF  
MAKING THE SAMEThomas P. Camp, Arlington Heights, Ill., assignor  
to United States Gypsum Company, Chicago,  
Ill., a corporation of IllinoisNo Drawing. Application March 1, 1946,  
Serial No. 651,381

9 Claims. (Cl. 154—86)

1

This invention relates to sheets or boards having a protected decorative surface, and also relates to methods of producing said boards or sheets. It relates particularly to decorated wallboards having a cementitious core.

Wall boards having a surface of decorative value have been produced for a number of years. These, principally, were made in patterns simulating wood and are sometimes known as "grain boards." Two general methods of manufacture have been employed. The first method of applying a decorative surface was to adhere to the regular paper surface of the dry gypsum or other board a sheet of paper bearing the desired pattern protected by a water and oil resistant film of lacquer. This sheet was applied to the gypsum board, for example, after it had been formed, dried and cut into sheets. This was an expensive procedure due to the extra handling of the boards, extra breakage, the cost of extra paper, etc.

The second method consisted of the application of a decorative pattern to the regular paper liner of the board before the board was formed, and then forming the board, cutting and drying it in the customary manner. This eliminated the objections of extra handling and extra paper, but yielded a product whose decorated surface was not water resistant. Furthermore it could not be varnished or otherwise finished without preliminary protective measures, either after drying or before erection of the board.

It is not desirable to ship a decorated board with a surface which is not cleanable or washable because of the possibility of defacing it during shipment or erection. Furthermore a decorative surface paper of prior art after passing through the drying kiln, does not take varnish or stain properly since the varnish, etc., strikes through or penetrates the surface, forming "oil spots." The application of a protective coating after drying the board, while effective, is obviously slow, laborious and expensive.

The greatest difficulty connected with the pre-decoration of the paper liner before formation into a board is the passage of moisture out through the water resistant protective coating during the drying of the board. These water resisting sized surfaces ordinarily prevent the passage of moisture through them, which either results in the blowing off of the surface paper in the kiln, or in so increasing the drying time that the production rate is decreased to a prohibitive low speed. In addition, since but one side is ordinarily decorated, the difference in the nature

2

of the two surfaces of the board frequently results in warping during the drying operation, thus causing serious difficulty in the kiln.

5 An object of the invention, therefore, is to provide a decorated sheet or board having a protected surface suitable for washing.

Another object of the invention is to provide a sized decorated board surface which after passing through the drying kiln, will resist the striking through of varnishes, stains, etc., which are subsequently applied.

A further object of the invention is to provide a gypsum board with a protected decorative surface which is economical to produce.

15 A still further object of the invention is to provide a practical method of producing such a decorated board or sheet; also to improve decorated sheets or boards and their methods of manufacture in other respects hereinafter specified and claimed.

It has been found that certain plasticized protein solutions and emulsions containing them in combination with the process of making a board will form a film on the paper which, although 20 water resistant and well suited as a varnish undercoater, will nevertheless permit the passage of moisture or steam therethrough during the drying of the boards.

Normally, a person skilled in the art of making gypsum wall board would expect that the application of a coating to one surface of a wet plasterboard would during the drying operation cause blistering and peeling. This is obvious 30 when it is considered that the moisture within the core would have only one avenue of escape; i. e., the surface that is not treated. If the drying process is pushed too rapidly there is a possibility that the moisture may attempt to escape as rapidly as possible and would be prevented at the interface of the coated sheet and the core. The moisture being present in the form of steam at the interface of the coated paper and the core would have a marked tendency to develop blisters and cause peeling.

40 However, in attempting to produce a satisfactory grainboard, it was found, quite contrary to natural expectations, that a coating of the type given below was very satisfactory and did not cause any warping, peeling or blistering in the finished product. It not only allowed uniform evaporation of the moisture through both surfaces of the wet plasterboard in the kiln, but also gave a vastly improved product.

45 As an illustration, but not as a limitation of the principles of this invention the method of

placing a decorative woodgrain appearance upon one of the paper surfaces of a gypsum wallboard will be described in detail. Gypsum wallboard, stated succinctly, consists of a core containing rehydrated calcined gypsum with additives and having firmly attached thereto on each side a layer of heavy paper known at times as a liner. It is not, however, intended to limit the application of this invention to a gypsum wallboard alone as it can obviously be applied to any type of board having one or more enclosing paper liners and a wet core.

The liner consists of several plies or sheets formed on a multi-cylinder paper making machine. Generally the outermost plies are formed from a stronger fiber so that the liner possesses adequate strength. In addition, one of the outer plies may consist of manila stock to provide a surface suitable for decoration. The paper to be used may also be supplied by the paper mill with the final or finish liner colored to a suitable shade for the type of wood graining which is to be applied upon it. For example, if the finished surface is to be a birch-like effect it will be light in color; if it is to be a walnut, it will be darker in color.

After the paper has been formed and dried it is ready for the application of the woodgrained effect. This can be accomplished in a number of ways well known to the art. One method is to print the grained effect on the paper using a roll or rolls, the surface or surfaces of which contain the impression of the graining effect it is desirable to produce. The appropriate color of ink is used for the printing. It is not intended to limit this invention to this pattern or color for obviously any pattern or color may be printed or otherwise transferred to the surface to be decorated.

When the decoration has become sufficiently dry to permit handling, a coating of a special film forming material is applied and permitted to dry. When dry this material is quite resistant to moisture penetration.

After the sizing has been thoroughly dried, the paper is wound into rolls, whence it is transported to the board forming machine and made into a board in the regular manner. This process consists of forming a bottom and top layer of paper so as to enclose a plaster core containing calcined gypsum and water by means of master rolls. The board, after the gypsum core has set up, is cut into the lengths desired and then passed through a drying kiln. The kiln may be heated by direct heat from a gas burner, from high pressure steam coils, or by other means. A slight adjustment may have to be made in the kiln conditions in order to properly dry the new material. These adjustments can readily be made by those familiar with the manufacture of wallboard.

The appearance of the product formed by this improved process will be found to be as good or better than that formed by the method now being used. The decorative surface of the board will be superior in its ability to take a varnish and there will be no danger of a separation of the grained surface from the base paper. In addition, the cost and difficulty of manufacture will be greatly reduced.

It has been found that a number of materials in an aqueous solution may be used as a basis for the special protective film. Casein, vegetable protein, glue, blood, albumen, etc. are some that can be readily used. They may be combined with

plasticizers such as urea, dicyandiamide and ethyl carbamid together with insolubilizing agents or tanning agents such as hexamethylenetetramine, formaldehyde, alum, chrome tanning agents. Likewise these water solutions may be converted into an emulsion with various oil type varnishes, oil modified alkyd resins, etc. When this is done, it is important that the solutions be in the continuous phase and the other ingredients in the discontinuous phase.

An example of a clear coating which is satisfactory for the purpose intended is as follows:

A casein paste is made according to the following formula:

|        | Lbs. |
|--------|------|
| Casein | 220  |
| Water  | 600  |

The casein is soaked in the water for about 25 minutes at room temperature and to this is slowly added 60 lbs. of borax dissolved in 420 lbs. of hot water. This mixture is cooked for 30 minutes at 170° F. and is then cooled and ready for use. The coating applied to the paper is made by mixing together the following ingredients:

|                                  |
|----------------------------------|
| 10 gallons above casein solution |
| 6 lbs. urea                      |
| .6 lbs hexamethylenetetramine    |
| 2½-3½ gal. water                 |

The urea and hexamethylenetetramine are dissolved in the water and then slowly stirred into the casein solution. It is important that the stirring be complete in order to prevent the formation of lumps.

The above quoted equivalent materials of course cannot be substituted directly in this formula, but must be used with the proper solvent and in the proper amount as determined by the nature of the paper and the equipment used for applying the solution:

As a further illustration which is not to be construed as a limitation of the principles underlying this invention, it is possible to use oil modified alkyd resins in an emulsion form. For instance to the above casein solution, may be added the following reacted alkyd resin mixture:

|                              | Percent |
|------------------------------|---------|
| 50 Soya bean oil fatty acids | 50      |
| 40 Phthalic anhydride        | 40      |
| 10 Glycerol                  | 10      |

The alkyd resin is emulsified with the aid of ammonia or some other volatile alkali and then stabilized with a casein solution. The amount of casein is approximately 10% of the dry weight solids. The alkyd emulsion generally contains about 50% by weight of solids.

It will readily occur to those familiar with the art of forming a wallboard having a decorative surface that many modifications can be made in the details of procedure in carrying out this process and still be within the scope of this invention. For example, it is possible to have the entire portion of the enclosing paper liner which is the base for the decoration, colored to the shade advisable for the particular effect desired instead of the top liner alone as suggested. Also it may only be necessary to apply this base color as a stain to the paper surface before application of the decoration. It is possible to apply a sizing layer between the base color and the decorated layer, or to the paper before applying the base stain. The coating, if desired, may be pigmented to produce a solid color. It also is

70  
75

obvious that the coating may be applied in any of the well known ways. It may be advisable to apply a surfacing material over the top sizing coat after drying and still not digress from the essence of this invention which is the formation of a decorated surface directly upon an enclosing paper liner of a wallboard in such a way that water or water vapor may pass therethrough during drying but which when cooled will be water resistant and suitable for the application of varnish or other decorative material in the field without discoloration of the surface.

Though the above illustrates but one of the many modifications, extensions, adaptations and variations possible, it is not intended to be limited to the same, since it is possible to be still within the spirit and scope of the principles of this invention as defined in the hereunto appended claims.

I claim:

1. The method of producing decorated gypsum board, which comprises applying a decorative pattern and a protein base coating material to a surface of a sheet of paper, drying said coated and decorated sheet, applying said dried decorated and coated paper to one surface of a plastic slurry of gypsum base core material having a substantial proportion of water, forming a laminated board therefrom and subjecting said board to an elevated drying temperature so as to expel at least part of said water from said board as vapor through said coated and decorated surface.

2. The method of producing a decorated surface gypsum board, which comprises applying a protein coated paper sheet to the wet gypsum board, the said protein selected from the group of casein, soya bean, peanut and zein, and subjecting said board to an elevated drying temperature to expel water as vapor through said sized and decorated surface without formation of blisters and peeler.

3. The method of producing a decorated gypsum board, which comprises applying the reaction product of casein and borax cooked at 170° F. for thirty minutes to a decorated sheet of vapor pervious flexible material, drying the said coated sheet, applying said sheet to a moist gypsum board, and subjecting said board to an elevated drying temperature to cause water vapor to be expelled from said board through said sheet.

4. The method of producing a decorated gypsum board, which comprises applying a pigmented coating solution of casein, an alkali, and a flexibilizer to a decorated sheet of vapor pervious flexible fibrous material, drying said coated sheet, applying said sheet to a moist gypsum board, and subjecting said board to an elevated drying temperature to cause water vapor to be expelled from said board through said sheet.

5. In the process of producing a decorative surface on a gypsum wallboard, the steps of placing a moistened cementitious core plastic mix on the uncoated side of an inverted sheet whose surface is decoratively coated, said coating comprising a protein emulsified alkyd resin and a pigment, placing on said moistened cementitious core plastic mix a cover sheet, and simultaneously pressing the said lamination to desired thickness, hardening the said moistened cementitious plastic mix by allowing it to stiffen and set without disturbance to a hard wet core in the lamination, cutting the said hardened lamination to desired size, inverting the cut lamination to expose the coated surface and drying said cut lamination in a kiln at a temperature sufficiently high to remove excess of said moisture from said core and said coating emulsion, whereby when the said laminated wallboard is dry a washable and decorative surface is obtained on said wallboard.

10 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000

6. A gypsum wallboard comprising a cementitious core and covering sheets, at least one of said covering sheets coated with the reaction product of a protein solution cooked at a temperature of not less than 170° F. and not more than 210° F. for a time of not less than twenty minutes; the said coated liner characterized by its ability to resist penetration of oil and varnish stains and also provide a washable and cleanable surface.

7. In the product of claim 6, wherein the said protein is selected from the group consisting of casein, albumen, soya bean, peanut and zein.

8. In the product of claim 6, wherein the said protein is flexibilized with a reagent selected from the group of urea, glycerine, dicyandiamide, and ethyl carbamid.

9. In the product of claim 6, wherein the said protein is water insolubilized with a reagent selected from the group of hexamethylene-tetramine, formaldehyde, alum, soluble chromates of alkali metals and ammonium.

THOMAS P. CAMP.

#### REFERENCES CITED

The following references are of record in the file of this patent:

#### UNITED STATES PATENTS

| Number    | Name             | Date           |
|-----------|------------------|----------------|
| 1,780,375 | Bradley          | Nov. 4, 1930   |
| 1,914,345 | Roos             | June 13, 1933  |
| 2,176,981 | Smith et al.     | Oct. 24, 1939  |
| 2,257,281 | Scholz           | Sept. 30, 1941 |
| 2,272,057 | Cheetham         | Feb. 3, 1942   |
| 2,352,553 | Lefebure         | June 27, 1944  |
| 2,409,630 | Heritage et al.  | Oct. 22, 1946  |
| 2,427,879 | Robertson et al. | Sept. 23, 1947 |